

# UNITED STATES PATENT OFFICE.

CHARLES KELLNER, OF GOERTZ, AUSTRIA-HUNGARY.

## METHOD OF SIZING PAPER.

SPECIFICATION forming part of Letters Patent No. 352,759, dated November 16, 1886.

Application filed April 23 1886. Serial No. 199,888. (No specimens.)

*To all whom it may concern:*

Be it known that I, CHARLES KELLNER, of Goertz, in the Empire of Austria-Hungary, have invented certain new and useful Improvements in Methods of Sizing Paper, of which the following is a specification.

This invention relates to an improved process of sizing paper, whereby the paper is not liable to assume a yellowish tint, as it does when sized in the ordinary manner.

The invention is specially designed for sizing paper made from ground wood pulp and sulphite cellulose, so that it assumes and retains a clear white color. The brownish-yellow tint which the paper made from wood pulp assumes after a certain time is caused by the size employed, which is produced by the precipitation of ordinary resin soap with aluminium sulphate.

My invention consists of a process of sizing paper by mixing the pulp, first, with a resin soap and precipitating the same with a sulphite salt—such as magnesium or aluminium sulphite, or calcium, magnesium, or aluminium bisulphite—or first with a sulphite salt and then with a resin soap.

In carrying out my invention ordinary colophony may be used in making resin soap therefrom, which soap is mixed with the pulp, after which one of the sulphite salts mentioned is added. The sulphite salts are lower in price than aluminium sulphate, and have the further advantage that, owing to the bleaching action of the sulphurous acid, the paper assumes and retains a perfectly white color, without being liable to change to a yellowish tint. The proportions used are those usually employed in sizing paper of this kind.

The advantages of my improved method of sizing paper are, first, that the sulphite salts can be easily produced by conducting the scrubbed and washed sulphurous acid through a tank containing resin soap, or the carbonate of the respective gases and water, which is cheaper than the use of the ordinary aluminium sulphate; secondly, owing to the influence of the sulphurous acid the wood pulp contained in the paper is rendered whiter and prevented from assuming a yellowish color, either on the drying cylinders or later, because the sodium sulphite, which is formed by the resin soap, resists any tendency to reduction; thirdly, in the presence of the sulphurous acid the resin size is precipitated even from inferior, and consequently cheaper, resin soap in a nearly colorless or whitish color; fourthly, the sulphite cellulose is continually kept in contact with salts which, by their reducing tendency, prevent the coloring of the resin size; and fifthly, the sulphite combinations act simultaneously as bleaching agents, so as to dispense with the necessity of bleaching with chlorine.

Having thus described my invention, I claim as new and desire to secure by Letters Patent—

The process herein described of sizing paper, which consists in mixing resin soap with the pulp and precipitating the resin size by a sulphite salt, substantially as set forth.

In testimony that I claim the foregoing as my invention I have signed my name in presence of two subscribing witnesses.

CHARLES KELLNER.

Witnesses:

GEORGE MARTIN,  
JOSEF HEIDLY.